

## UNITED STATES PATENT OFFICE

2,168,563

## NITROSTARCH EXPLOSIVE

Clyde Oliver Davis, Woodbury, N. J., assignor to  
E. I. du Pont de Nemours & Company, Wil-  
mington, Del., a corporation of Delaware

No Drawing. Application March 8, 1938,  
Serial No. 194,606

4 Claims. (Cl. 52—11)

The present invention relates to the production of improved explosive compositions, and, particularly, to such compositions wherein nitrostarch serves as a sensitizing ingredient.

As is well known, the use of nitrostarch as an explosive ingredient has been attended with so many disadvantages as to discourage its use. An outstanding disadvantage of the use of nitrostarch in explosives has been the extreme insensitivity to propagation of the resulting compositions. Nitrostarch also has the disadvantage that it is highly sensitive to accidental initiation by means of sparks, friction, and shock. A further undesirable feature has been the difficulty in manufacturing and handling nitrostarch and the explosives containing same due to the extreme dustiness of these materials.

The object of the present invention is a new and improved nitrostarch explosive. A further object is a nitrostarch explosive with improved sensitivity to propagation, in which ammonium nitrate is an important constituent. Another object is a nitrostarch explosive of improved stability against unintentional initiation by impact. An additional object is a new and improved process for producing explosives comprising nitrostarch and ammonium nitrate. Other objects will be apparent from the following detailed description of my invention.

I have found that the foregoing objects are accomplished and the foregoing disadvantages overcome by the process of my invention which comprises dissolving ammonium nitrate in substantially anhydrous liquid ammonia, dispersing in said solution, nitrostarch as a sensitizing ingredient, expelling the free ammonia and thereby forming a product in which the nitrostarch is dispersed in solid ammonium nitrate, the latter compound being a continuous phase. Preferably an imperforate form of nitrostarch will be employed, which will be non-absorbent and free from pores and cavities, since a dispersion of the nitrostarch in the ammonium nitrate is desired, and not saturation of the sensitizer with the ammonium nitrate solution prior to solidification.

While many different methods of carrying out my invention may be employed, the following examples are illustrative of desirable methods of procedure.

50 *Example 1*

850 grams of ammonium nitrate was introduced into a jacketed graining kettle equipped with agitation means. 150 grams of nitrostarch was added, and the mixer was closed. 250 grams

of anhydrous liquid ammonia was then run into the graining kettle and the agitation of the mixer was maintained during the solution of the ammonium nitrate. The free ammonia was then expelled by heating the charge to 30–35° C., with final evacuation under reduced pressure. The agitation was continued during the drying, so that a dry, loose product resulted, comprising minute regions of nitrostarch disseminated within crystals of ammonium nitrate. The explosive 10 composition was punched into cartridges of such density that 153 cartridges were contained in a 50-lb. case. This explosive showed a sensitivity of 7 inches by the double-cartridge test, where full sticks were used without removal of 15 crimped ends, and a velocity of detonation of 3670 m/sec.

Example 2

830 grams of ammonium nitrate was introduced into a jacketed graining kettle in the same manner as in Example 1. 150 grams of nitrostarch was then added, together with 20 grams of a foam-suppressing mixture, and the mixer closed. 250 grams of anhydrous liquid ammonia was run into the graining kettle, and the incorporation of ingredients and preparation of the dried product were carried out as in Example 1. The finished explosive composition was punched into cartridges running 148 to the 50-lb. case, and showed a sensitivity of 6 inches, and a velocity of 3830 m/sec.

Example 3

400 grams of ammonium nitrate was introduced into a jacketed graining kettle, as in Example 1, together with 80 grams of nitrostarch. Sufficient anhydrous liquid ammonia was run into the graining kettle to dissolve all the ammonium nitrate, and form a substantially saturated solution, and 520 grams of coarsely granulated ammonium nitrate was also introduced into the kettle. After incorporation with the ingredients, the free ammonia was expelled as in Example 1, and a dry product obtained. This explosive composition was punched into cartridges such that 145 per 50-lb. case resulted. The explosive showed a sensitivity of 1 inch by the double-cartridge test and a velocity of detonation of 1345 m/sec.

The compositions prepared according to my invention and illustrated in the foregoing examples may be employed as explosives either by themselves, or blended with other materials to obtain the desired oxygen balance, as well as to control other explosive properties. For instance,

20

25

30

35

40

45

50

55

other conventional ingredients may be added, such as nitrate of soda and the common combustibles; viz., ground coal, starch, and meals. It will be understood that various degrees of 5 sensitiveness may be obtained, depending on the relative proportions of ammonium nitrate and nitrostarch employed. In many cases it may be desirable to introduce a so-called "foam-prevention" agent to suppress foaming during the 10 expulsion of the free ammonia. As examples of such agents, I may cite oleic acid or lard oil.

The present process brings many advantages in the preparation of such nitrostarch compositions and allows the use of proportions of materials which would not be possible otherwise for 15 obtaining the desired properties.

The outstanding advantage of my invention is the fact that nitrostarch explosives having highly 20 enhanced sensitiveness to propagation are prepared thereby. These explosives have a further advantage over nitrostarch explosives of the prior art in that they exhibit a decreased sensitiveness to unintentional initiation by sparks, friction, and incidental shock. Furthermore, the preparation 25 of nitrostarch explosives by my improved ammonia process eliminates all dust during manufacture and the hazards attendant therewith.

These advantages of enhanced sensitiveness to propagation and stability against impact are 30 demonstrated quantitatively in the following table.

| 35 | Ingredients and properties                   | A                                    | B                                                               |
|----|----------------------------------------------|--------------------------------------|-----------------------------------------------------------------|
|    |                                              | Incorporation by conventional method | Incorporation according to the process of the present invention |
| 1  | Percent nitrostarch.....                     | 15                                   | 15                                                              |
| 2  | Percent ammonium nitrate.....                | 85                                   | 85                                                              |
| 3  | Full stick sensitiveness test in inches..... | 2                                    | 6                                                               |
| 4  | Stability against impact.....                | 120                                  | 995                                                             |

The above tabulation compares two nitrostarch explosives with respect to sensitiveness to propagation and stability against impact. These two explosives have identical compositions but differ in properties as the result of difference in methods of preparation. The nitrostarch explosive of column "A" consists of 15% nitrostarch and 85% 45 ammonium nitrate incorporated by intermingling the particles of these two ingredients in conventional fashion. The nitrostarch explosive of column "B" consists of the same ingredients in the same proportions, but these ingredients have 50 been incorporated by dispersion in liquid ammonia according to the process of the present invention.

The widely divergent properties resulting from these two methods of incorporation are shown in the horizontal columns 3 and 4. The sensitiveness 55 of the explosives to propagation was readily determined by the full stick sensitiveness test. Horizontal column 3 indicates the results of this full stick sensitiveness test as applied to both compositions. This test may be defined as the maximum width of air gap across which propagation 60 of the detonation wave will occur between full sticks or cartridges placed in line lengthwise without removal of the crimped ends. This distance is expressed in inches in the foregoing table. Thus, it is shown that the nitrostarch explosive 65 according to the present invention is more sensitive to propagation than the explosive of the art, in a ratio of 6 to 2.

Horizontal column 4 shows the results of the

test for determining stability against initiation by impact. In this test a weight is permitted to fall from a measured height upon the powder to be tested, and the minimum height is determined at which the powder fails to detonate in 10 falls 5 of the weight. The result is expressed in the terms of the "impact", defined as the height in inches multiplied by the weight in pounds.

In the application of this test to the foregoing powders, it will be noted in column 4 of the table 10 that the nitrostarch explosive according to the present invention, exhibits increased stability over the explosive of the art in a ratio of 955 (impact) to 120.

The importance of these enhanced properties 15 of my explosive thus quantitatively demonstrated, will be clear to any explosive technologist.

A further advantage resulting from my process of preparation comes in the better control 20 of sensitiveness of the finished explosive to intentional initiation. As prepared by my invention, the compositions have an excellent degree of sensitiveness such as has been obtained by no previous method of preparation. By use of my 25 method, a given sensitiveness value can be obtained by the employment of smaller percentages of nitrostarch, and at the same time greater uniformity of product results.

In my co-pending application Serial No. 194- 30 551, filed March 8, 1938, I have disclosed my ammonia process as applied to the manufacture of explosive compositions generally. It will be understood that, in the present application, I 35 intend to claim only a preferred type of explosive; namely, an improved nitrostarch explosive as prepared by the ammonia process.

Many different embodiments of this invention 40 may be brought about without departing from the spirit and scope thereof. I wish, therefore, 45 to be limited only by the following patent claims.

I claim:

1. A nitrostarch explosive comprising particles 45 of nitrostarch dispersed within crystals of ammonium nitrate, having an enhanced sensitiveness to propagation and decreased sensitiveness to unintentional initiation as the result of crystallization from substantially anhydrous liquid ammonia.

2. The process of preparing a nitrostarch explosive of improved sensitiveness to propagation and decreased sensitiveness to unintentional initiation, which comprises dissolving ammonium nitrate in substantially anhydrous liquid ammonia, dispersing nitrostarch in said solution, 55 and expelling the free ammonia therefrom.

3. The process of preparing a nitrostarch explosive of improved sensitiveness to propagation and decreased sensitiveness to unintentional initiation, which comprises dissolving ammonium 60 nitrate in substantially anhydrous liquid ammonia, dispersing nitrostarch in said solution, and vaporizing the free ammonia to produce a solid dispersion product wherein ammonium nitrate is a continuous phase.

4. The process of preparing a nitrostarch explosive of improved sensitiveness to propagation, which comprises dissolving ammonium nitrate in substantially anhydrous liquid ammonia, dispersing nitrostarch in said solution, together 65 with a small percentage of a foam-suppressing agent, and expelling the free ammonia therefrom.

CLYDE OLIVER DAVIS.